

# United States Patent Office.

FRANCIS ELLERSHAUSEN, OF MONTREAL, CANADA EAST.

*Letters Patent No. 77,469, dated May 5, 1868.*

## IMPROVED PROCESS OF CONVERTING CAST IRON INTO CAST STEEL AND MALLEABLE IRON.

The Schedule referred to in these Letters Patent and making part of the same.

### TO ALL WHOM IT MAY CONCERN:

Be it known that I, FRANCIS ELLERSHAUSEN, of Montreal, Canada East, have invented a new and improved Process for Converting Cast Iron into Cast Steel and Malleable Iron; and I do hereby declare that the following is a full, clear, and exact description thereof, which will enable others skilled in the art to understand the same.

This invention relates to a new process for converting cast iron into malleable iron or cast steel, and consists in bringing the carbon contained in the molten cast or pig iron in contact with oxygen contained on the surface of a cold or hot solid substance or substances.

The distinguishing feature between this, my invention, and that known as the Bessemer process is, that in the latter the carbon contained in the molten cast or pig iron is brought in contact with and consumed by the oxygen, which is formed by forcing vaporous substances through the liquid metal, while, in my process, the oxygen is held on the surfaces of substantial or solid bodies, and is formed thereon, preparatory to the decarbonizing process.

It is well known that carbon at a white heat cannot exist in the presence of oxygen, as it is at once burned when brought in contact with the same. The rapidity of combustion depends on the temperature of both the carbon as well as the oxygen, and on their proportionate quantities.

The apparatus for bringing the carbon contained in the iron into contact with the oxygen held on the surface of a solid substance may be of suitable description, and I do not bind myself to the use of any particular apparatus. The following would, perhaps, be the simplest apparatus:

In a converter, of suitable form, are placed, in a vertical-position, coils of sheet iron, the same being so rolled that the spiral spaces formed in them will be just large enough to allow liquid cast iron, (carburet of iron,) flowing through these spaces, to be brought in contact with the required quantity of oxygen, (oxide of iron,) on the surfaces of the sheet metal, to produce the required quality of steel or malleable iron.

The converter is heated to a suitable temperature in suitable manner, it being preferable to bring the sheet curlings to a white heat, and to continue for a sufficient length of time to insure their complete oxidation. When this is accomplished, a sufficient quantity of molten cast or pig iron is poured into the top of the converter, to unite with the oxide of iron already formed on the curlings, and to thereby have the carbon consumed, or so much of it as is requisite to produce the desired quality of steel or malleable iron.

It will be evident, from the manner in which the sheet-iron curlings, afterwards converted into oxide of iron, are placed in the converter, that a large surface of oxide of iron is exposed, within a comparatively small space, to contact with the molten cast iron, uniting the particles of each in close conjunction, causing a rapid combustion throughout the entire mass, which increases the temperature to such a degree as to cause a complete conversion while the metal is in fluid state.

Instead of the iron shavings or curlings, other solid oxides may be used, in either a hot or cold state. In either case, purifying, decarbonizing, or steel-improving agents may be deposited in the converter, in order to facilitate the combustion or purification, as may be desired.

Having thus described my invention, what I claim as new, and desire to secure by Letters Patent, is—

1. Converting cast or pig iron into cast steel or malleable iron, by bringing it, in a liquid state, in contact with hot or cold solid oxides, substantially as herein specified.

2. Bringing to an instantaneous uniform contact, at a sufficient heat, on a sufficiently large hot or cold surface of pure oxide, the carbon contained in molten cast iron, so as to cause a rapid violent combustion of the carbon, substantially as described.

The above specification of my invention signed by me, this 4th day of April, 1868.

FRANCIS ELLERSHAUSEN.

Witnesses:

WM. F. McNAMARA,  
ALEX. F. ROBERTS.